

A. R. FRANK.  
PROCESS OF PRODUCING NITROGEN COMPOUNDS.  
APPLICATION FILED MAR. 23, 1908.  
987,674.

Patented Mar. 21, 1911.



Witnesses

Geo. A. Ryne.  
W. Maxwell

Inventor

A. R. Frank by  
Wickinson Fisher &  
Witherspoon

Attorney

# UNITED STATES PATENT OFFICE.

ALBERT RUDOLPH FRANK, OF HALENSEE, NEAR BERLIN, GERMANY, ASSIGNOR TO  
THE FIRM OF SOCIETA GENERALE PER LA CIANAMIDE, OF ROME, ITALY

## PROCESS OF PRODUCING NITROGEN COMPOUNDS.

987,674.

Specification of Letters Patent. Patented Mar. 21, 1911.

Original application filed March 13, 1907, Serial No. 362,086. Divided and this application filed March 23, 1908. Serial No. 422,779.

To all whom it may concern:

Be it known that I, ALBERT RUDOLPH FRANK, a subject of the German Emperor, and resident of Halensee, near Berlin, Germany, have invented certain new and useful Improvements in Processes for Producing Nitrogen Compounds from Carbids, of which the following is a specification.

The present invention relates to a process for producing nitrogen compounds from carbids, of the character illustrated in the following equation, in which the calcium compound is cited merely as an illustration:



This application is a division of my former application Serial Number 362,086, filed March 13, 1907.

In the production of nitrogen compounds by the reaction of nitrogen with carbids, as for example, the carbids of the alkalies or alkaline earths, it has been ascertained that it is not necessary for the process that the entire mass of the carbid be brought to the temperature necessary for the reaction by supplying external or intrinsic heat to the entire mass; but that it suffices if this temperature be produced at one place in the mass, when the reaction then continues spontaneously throughout the entire mass. A preliminary condition however is that the reaction temperature of from about 800° C. to 1100° C. be actually attained at this one place.

In accordance with the present invention the process may be carried out in several ways, of which the following are examples:

The ignition at one place may be produced by a convenient heating means evolving heat by chemical reaction, which will raise the temperature at that place to the temperature required for the conversion of the carbids, whereupon the conversion will proceed spontaneously throughout the mass, sufficient nitrogen being present to effect the conversion. The production of a temperature sufficiently high for the absorption of nitrogen by the carbid at one place or point of the carbid by means of said chemical heating in order to raise the carbid at this one place to the proper ignition temperature may be accomplished:—(a) by means of a primer comprising an explosive mass or

the like; or (b) by means of substances reacting with carbid with the production of 55 the necessary heat, which substances, if in the solid state such as chlorate of potassium, nitrate of alkali, etc., may be added to the carbid at the place of ignition; while if the substances are gaseous, such as chlorin or 60 oxygen, the same may be added to or employed with the first portions of the nitrogen that are led to the carbid until the ignition has taken place; or (c) the requisite 65 temperature may be produced by substances such as magnesium or aluminium which, when mixed with the carbid at the place of ignition, react with the nitrogen with the 70 production of the desired heat. After the ignition has produced a temperature sufficient to cause a further absorption of the nitrogen, the latter is further supplied, and it will continue to be absorbed with a further development of heat so that the continued supply of nitrogen will cause the absorption to proceed spontaneously throughout the mass.

Referring to the accompanying drawing forming a part of this specification in which the figure represents a diagrammatic sectional view of an apparatus suitable for carrying out my invention, 1 represents a furnace or other suitable heating means; 2 a suitable container for the reacting substances; 3 an opening through which the 85 said substances may be introduced; 4 an inlet for the reacting gas, or gases; 5 an outlet for the same; and 6 an outlet for the finished product; it being, of course, understood that this apparatus merely illustrates 90 one example of a means by which the invention may be carried out.

The following example will explain how the present invention can be put into practice. For example, the heating by chemical agencies may be accomplished by mixing with the nitrogen such gases as will cause a local high temperature by reaction with the carbid, when the latter is heated to a moderate temperature below the temperature of reaction. 95 Such gases are oxygen, air, chlorin or the like. To carry out the process by this means, a suitable proportion of such a gas is mixed with nitrogen and brought into reaction with the carbid, whereupon the temperature is raised to that required for the 100 105

conversion, and sufficient nitrogen being supplied the reaction will continue without further heating until the entire mass is converted. Or, if desired, the temperature necessary for starting the reaction may be obtained by the addition to the carbid of substances such as powdered aluminium or magnesium, which will serve to start the reaction locally, and upon the nitrogen being supplied in proper quantity, the reaction will propagate itself throughout the entire mass.

In carrying out the invention the nitrogen may be supplied at a pressure equal to 15 or above that of the atmosphere, or it may be sucked into the receptacle at a pressure below that of the atmosphere.

The carbid may be used at any temperature below about 800° C. to 1,100° C., the temperature which is necessary for the absorption of the nitrogen; for the heat produced by such absorption will be sufficient to produce the reaction in the surrounding parts of the carbid. The nitrogen may be introduced at the ordinary temperature, or it may be heated, while the carbid with which it is brought into contact, may be either cold or warm. It is evident that the higher the temperature of the reacting bodies (nitrogen or carbid) the easier and more quickly will the absorption of the nitrogen proceed. If carbid or nitrogen or both are employed in a warm state, it is not necessary, according to the present invention, to heat these bodies to a temperature equal to or higher than the absorption temperature, since as has been shown by us, the heat produced by the absorption of the nitrogen itself, is sufficient to cause the reaction to proceed in and through the reacting mass. The progress of the reaction, however, is accelerated by employing the nitrogen or the carbid or both at a temperature higher than the ordinary temperature, 45 although the reaction proceeds without raising these bodies to an elevated température.

In all cases, there may be employed either pure or commercial carbids, or carbids mixed with other materials, particularly with such materials as are adapted to facilitate or favorably influence the promotion of the absorption of the nitrogen, while absorption, as above stated, takes place according to the present invention through the heat produced by said absorption itself. Such other materials or additional substances may be *e. g.* cyanamid of calcium ("lime-nitrogen"), oxides of alkaline earths or of other metals or salts thereof, such as chlorids, sulfates, sulfids, or any suitable materials especially adapted to produce a loosening of the carbid mass. Carbonaceous materials are especially adapted for this purpose, because they by becoming carbonized form channels or pores in the mass,

which channels or pores enable the nitrogen to penetrate easily throughout all the portions of the mass.

The carbid may be employed either in the powdered state or broken into lumps. Further, the carbid employed need not be completely formed carbid but may be in the form of its components, as for example, a mixture of oxids and carbids or other salts of alkalies and alkaline earths and carbon or any carbonaceous substances derived from carbon; or as a mixture of metals and carbon, with or without the addition of other organic or inorganic substances, provided these components do not contain compounds having a temperature of decomposition which in itself or in reaction with the other components is higher than the temperature of reaction when nitrogen acts on carbids.

It is to be clearly understood that the word "carbid" as used in this specification and in the claims, signifies and includes not only all pure carbids as such, but also carbids in the forms of their components, such as the mixture of oxids or other salts or metals with carbonaceous material, as indicated above.

The nitrogen employed may be either nitrogen as such or nitrogen in a combined state, such, for example, as ammonia, provided the temperature at which the nitrogen compound decomposes be lower than the temperature at which nitrogen reacts upon the carbid.

The nitrogen may be introduced into the carbid mass at the point where the absorption takes place, as above stated, and it may be further supplied in the direction in which this absorption proceeds, but the nitrogen may be also introduced in the opposite direction, so long as this gas passes through a portion of the mass which has not been acted upon or along the surface of the same toward the point where the absorption takes place. It is also to be understood that the word "nitrogen" as used in this specification and in the claims specifies and includes not only pure nitrogen as such but nitrogen mixed with other gases, vapors or substances, as well as nitrogen in the combined state, such as ammonia, for example.

I am aware that nitrogen compounds have hitherto been produced from carbids by the reaction of nitrogen upon carbids and I therefore do not claim such method or process broadly, but

What I claim is:—

1. The process of making a compound of nitrogen by reacting upon a carbid with nitrogen at a suitable temperature, which consists in admixing with a portion of one of the reagents a substance capable of chemically reacting upon either of the ingredients to develop heat sufficient to initiate the re-

action, supplying nitrogen as the reaction proceeds, maintaining the temperature and continuing the reaction throughout the mass to be converted.

5 2. The process of making a compound of nitrogen by reacting upon a carbid with nitrogen at a suitable temperature, which consists in mixing with a portion of the nitrogen a gas capable of reacting upon the car-  
10 bid to develop heat sufficient to initiate the reaction, supplying nitrogen as the reaction proceeds, maintaining the temperature and continuing the reaction throughout the mass to be converted.

15 3. The process of making a compound of

nitrogen by reacting upon a carbid with nitrogen at a suitable temperature, which consists in mixing oxygen with a portion of the nitrogen, supplying nitrogen as the reaction proceeds, maintaining the temperature and 20 continuing the reaction throughout the mass to be converted.

In testimony that I claim the foregoing as my invention, I have signed my name in presence of two subscribing witnesses.

ALBERT RUDOLPH FRANK.

Witnesses:

HENRY HASPER,  
WOLDEMAR HAUPT.